

## UNITED STATES PATENT OFFICE

EDWIN R. MILLRING, OF NEW YORK, N. Y., ASSIGNOR TO AMERICAN MACHINE & FOUNDRY COMPANY, A CORPORATION OF NEW JERSEY

## METHOD OF COATING METALS

No Drawing.

Application filed July 21, 1923. Serial No. 653,022.

This invention relates to the covering of metals with a metallic coat to protect them from the elements of oxidation and corrosion, such as exposure to the atmosphere, water, 5 sea water, salt solutions, acids, chemicals, industrial gases, etc., and the invention is applicable to the treatment of various metals, such as iron, steel, copper, brass, etc., in order to give them a protective coating.

10 The objects of the invention are to produce a protective coating which will be of the requisite thickness, hardness, and continuity, to withstand the effects of oxidation, corrosion, and abrasion, and the invention 15 consists primarily in a method of procedure involving the application to the metal to be protected, of a protective coating alloy in super-cooled or metastable condition.

The invention consists also in the application of such super-cooled protective alloy to metals having a previously applied protective base coat, in order to thicken such base coat, fill up and cover breaks or pin holes or other defects therein, and thus produce continuity of the same; in some cases to produce 25 a secondary metallic coat actually superimposed upon the base coat, a result not obtained by other methods on account of the alloying action between the first and second 30 coats; and to provide an outer hard coat well adapted to prevent abrasion.

The invention consists also of the improved alloy bath employed in carrying the method into effect.

35 It is known that certain metallic solutions, as well as non-metallic solutions, can exist in the liquid state at a considerably lower temperature than that at which the solid metal, alloy or substance would melt or become 40 entirely molten, or be in true liquid solution, and this condition is known as the super-cooled solution or metastable condition of the metal, alloy or substance, and, with certain metals, alloys and substances, 45 this metastable condition is rather pronounced. It is also known that, when certain alloys have been brought to a perfectly homogeneous liquid solution by the application of heat, and are allowed to cool, at a certain temperature one or more components of the al-

loys begins to freeze out. This temperature point is known as the liquidus for the particular alloy. When the alloy is allowed to cool further, it still exists in a partly solid and partly liquid condition until the temperature point is reached where the entire alloy has become entirely solid. This temperature point is known as the solidus of the alloy. When objects are immersed in certain alloys having these properties, and under these conditions, that is, in the metastable condition or at a temperature between the liquidus and the solidus, a precipitation, deposition, or crystallizing out of one or more of the components of the alloy occurs 55 on the surface of the metal surface of the objects, and such deposition, precipitation or crystallizing out increases the thickness of the coat and consequently its protective value, 60 and it also increases the continuity and hardness of the coat, so that the effect is to produce a coating possessing all of the properties which will best serve the objects and advantages sought. It is such a super-cooled 65 alloy that I employ in the treatment of metals to apply a protective coating, the said alloy being either applied directly to uncoated metals, or applied as a second coating to metals having a previously applied metallic base coat.

70 It is of course recognized that, in the case of alloys not possessing the above mentioned properties, or in the case of alloys possessing these properties under conditions other than herein described, such as at a higher temperature than the liquidus of the alloy, or at such a temperature as when the alloy is a perfectly homogeneous stable liquid, the advantages sought would not be obtained, and the coating so obtained would be much thinner and less continuous, thus possessing the 75 faults of the usual hot dipping process.

80 Examples of two alloys, electro-positive to iron, and exhibiting the above mentioned properties of a super-cooled solution are the 85 following:

1. Antimony 12.5%, bismuth 10.0%, lead 77.5%.
2. Antimony 12.5%, cadmium 5.0%, lead 82.5%.

55

60

65

70

75

80

85

90

95

100

The following is an example of an alloy having the above mentioned properties of a super-cooled solution but electro-negative to iron: Zinc 18%, cadmium 82%.

In practicing my invention, in applying a protective coating directly to uncoated metal, when employing an alloy for instance of antimony, lead and bismuth, the metal to be protected is first cleansed in any suitable and appropriate manner, as by heat treatment, 10 mechanical, chemical, or electrical means, and is fluxed with a suitable flux, such as zinc chloride or the like. The alloy bath is now prepared, the proportion of antimony not to exceed 15%, bismuth not to exceed 40%, and 15 the remainder lead; but I prefer that the ingredients shall be in the proportions first mentioned, viz., 12.5% antimony, 10% bismuth, and 77.5% lead. These ingredients are 20 reduced to molten condition and heated to a temperature of approximately 450° C. in order to bring about their complete fusion and to produce a true solution, thereby producing an alloy having a melting point of approximately 232° C. The temperature of the bath 25 is then lowered sufficiently to bring it to a super-cooled condition and producing a super-cooled alloy possessing the properties hereinbefore described. The cleansed and 30 fluxed metal is now immersed in this super-cooled bath, and receives on its surface a coating of the alloy, and on being withdrawn from the bath, it may be quenched in water or oil or other suitable quenching medium.

When employing an alloy of antimony, cadmium and lead, or of cadmium and zinc, as in the examples above given, which alloys have melting points respectively of 240° C. and 270° C., the method of procedure would 40 be the same as that just described, the bath being first heated to a temperature to produce a true solution of the ingredients, and then reduced in temperature to bring about its super-cooled condition.

Other alloys may be employed which possess the properties of a super-cooled solution, without departing from the limits of my invention, those above given being merely by way of example, and such as have been 50 found in practice to answer to a satisfactory degree the ends to be attained.

In the practice of my invention when applying a protective coating to metals having a previously applied metallic base coat, 55 the base coat may be galvanized tin, lead, copper or other metals or alloys, and the coat may be applied by the usual methods practised in the art, such as by hot dipping, spraying, electro-plating, etc. The metal with the 60 base coat applied, and after the base coat has set, is immersed in a super-cooled alloy bath prepared in accordance with my invention as hereinbefore described, with the result that the base coat will receive on its surface 65 a coating of this alloy, which being de-

posited under the super-cooled conditions described, will have the effect of increasing the thickness of the base coat, and will increase its hardness, and will cover up such defects or breaks or pin holes as may exist in the base 70 coat, and in this way will bring about a perfect continuity of the protective coating. In some cases the application of the super-cooled alloy to the previously coated metal, actually superimposes upon the base coat, a 75 secondary coat, which could not be brought about by other means on account of the alloying action which would take place between the first and second coats. While the super-cooled alloy may be applied directly to the 80 base coat after the latter has set as above described, yet it may in some cases and under certain conditions be desirable to quench the base coat with or immerse the same in a suitable flux solution to render the surface receptive to the super-cooled alloy.

While in the case of the application of a super-cooled alloy to previously coated metal, the base coat may be composed of various kinds of metals or alloys of the same as hereinbefore mentioned, I have found that a very satisfactory coating may be obtained in accordance with my invention by applying a super-cooled alloy of lead, antimony and bismuth or of lead, cadmium and antimony, to a base coat composed of lead, phosphorus and tin wherein the lead is in a proportion greatly predominating the other ingredients, and such as would be produced by mixing with ninety-seven (97) pounds of lead three (3) pounds or less of phosphor tin. A base coat of these particular ingredients has been found to adhere very tenaciously and closely to the metal to which it is applied, on account of the presence of the phosphorus therein, and by applying thereto a coating alloy in super-cooled condition, a protective covering for the metal is secured possessing in marked degree the properties above described with respect to thickness, hardness and continuity 100 and the consequent resistance to oxidation, 105 corrosion and abrasion.

Having thus described my invention, what I claim is:

1. The method of covering metal with a protective metal coating, which consists in applying to the metal a coating alloy in super-cooled condition.
2. The method of covering metal with a protective metal coating, which consists in immersing the metal to be coated in a super-cooled bath of an alloy.
3. The method of preparing a coating bath for metal, which consists in providing an alloy bath heated to a temperature at which the ingredients are in true solution, and reducing the temperature of the bath to super-cool the same to bring it to a metastable condition.
4. The method of covering metal with a

protective metal coating, which consists in applying a primary metal coating thereto, allowing said coating to set, and immersing the coated metal in a super-cooled alloy bath.

5. The method of covering metal with a protective metal coating, which consists in applying a primary metal coating thereto, allowing said coating to set, and immersing the coated metal in a super-cooled bath containing antimony and lead.

6. The method of coating metal with a protective metal coating, which consists in applying a primary metal coating thereto, allowing said coating to set, and immersing the metal in a super-cooled bath of an alloy 15 alloy of antimony, bismuth and lead.

7. The method of coating metal with a protective metal coating, which consists in applying a primary metal coating thereto, 20 allowing said coating to set, and immersing the coated metal in a super-cooled bath of an alloy of antimony, bismuth and lead in substantially the proportions specified.

8. The method of coating metal with a protective metal coating, which consists in applying a primary metal coating thereto, allowing said coating to set, and immersing the coated metal in a super-cooled bath of an alloy of 12.5% of antimony, 10% of bismuth, and 77.5% of lead.

In testimony whereof, I have affixed my signature hereto.

EDWIN R. MILLRING.

35

40

45

50

55

60

65